

Jan. 28, 1941.

R. C. JOHNSON ET AL

2,229,974

METHOD OF PRODUCING MINERAL WOOL

Filed Sept. 30, 1938



INVENTORS

Raymond C. Johnson, and  
Harold J. Rose  
by Christy and Wharton  
their attorneys

## UNITED STATES PATENT OFFICE

2,229,974

## METHOD OF PRODUCING MINERAL WOOL

Raymond C. Johnson and Harold J. Rose, Pittsburgh, Pa., assignors to Anthracite Industries, Inc., a corporation of Delaware

Application September 30, 1938, Serial No. 232,632

5 Claims. (Cl. 49—77.5)

This invention relates to the production of mineral wool and consists in a method, whereby materials not heretofore recognized to be sources of mineral wool may be resorted to for such production.

The accompanying drawing illustrates diagrammatically the method of the invention.

In an application for Letters Patent of the United States, Serial No. 223,687, filed August 8, 1938, Raymond C. Johnson has described the derivation of mineral wool from the ashes of industrial furnaces; and in a second application, Serial No. 232,609, filed on even date herewith, the said Johnson has defined the wastes of coal-mining and coal-washing operations as source materials for the production of mineral wool. The present invention recognizes all these sources, and consists in a method of dealing with any and all these materials with the production of mineral wool.

The practice of the invention involves the operation of a slagging gas producer. A slagging gas producer consists essentially of a refractory-lined furnace chamber of essentially cylindrical shape standing in vertical position, to which fuel is fed from above, and combustion-sustaining air from below, while steam is injected into the furnace charge at an intermediate point in the height of the furnace. The parts are so proportioned and arranged that a combustion zone is maintained at an intermediate portion of the vertical extent of the furnace chamber. The gas formed by the action of steam in the air-blown fuel bed consists chiefly of carbon monoxide and hydrogen. From the upper part of the furnace chamber the gas is drawn off; from below, the slag is discharged.

In practising the present invention the furnace is charged with material of the kind named above, typically the ash from an industrial coal-burning furnace. This ash is a heterogeneous mixture of unburned or partially burned fuel, together with inorganic, mineral residues that commonly include, in predominant quantities, alumina and silica. In physical condition it may range from dusty, friable and finely divided material to large hard clinkers.

The furnace being so charged, and being operated, the gas produced by operation is used as fuel to generate steam, and the steam so generated is employed to blow to the condition of wool the molten slag as it flows from the furnace.

Referring to the drawing, the furnace chamber is indicated at 1; its charging door at 2, and its slag-delivery orifice at 3. Air ports 4 are

diagrammatically indicated, through which combustion-sustaining air is blown into the furnace charge. Above the level of the air ports steam ports 5 are arranged, and through these the steam is injected that combines with the hot solid fuel to form the gaseous product described. Through ports 6 the producer gas is drawn off.

Adjacent the furnace 1 is arranged a boiler 7. This boiler is heated by the burning of the gas produced in furnace 1 and delivered through ports 6. In general, it will be necessary to burn no more than a part of the producer gas to generate steam for the blowing of wool; the surplus may be used for any other desired purpose. Adjacent the ash delivery 3 from furnace 1 is arranged a nozzle 8 and to this nozzle steam from boiler 7 is fed, and from the nozzle the steam is projected in a jet. The jet plays upon the escaping stream of molten slag, and blows it to wool, within the wool room 9.

Steam from boiler 7 may be delivered, not through nozzle 8 only, to blow the slag to wool, but to ports 5 also, to serve in the production of the gas, as already indicated. The injected steam not only serves to accomplish the reaction described; it serves also to control temperature, and to prevent sintering and clogging of the fuel bed above the combustion zone. The air that enters through ports 4 into the furnace is introduced under pressure, and to such end a blower 10 may be provided. Furthermore, the introduced air will be heated to high degree for its service, and, to such end, the producer gas, serving as already described, to heat the water in boiler 7 and so to produce steam for the operation described, may be made to serve further, in heating the air that is blown through ports 4 into the furnace. This also is indicated in the drawing. The degree to which the air is pre-heated will vary inversely with the combustible content of the furnace charge. The sensible or latent heat from the gases may be used to drive the blower 10 also.

The fuel ashes that are introduced into the furnace 1 may be introduced in the condition in which they come from the ash pit of the furnace in which they were formed, or they may be worked upon, in preparation for their further treatment. Large lumps may be broken; fines may be sifted out and otherwise disposed of. Or, the fines may be briquetted and returned to the mass. Additions may be made, either of fuel in solid or in liquid state (in case the ash is very lean in carbon content), or of flux (in case the ash is low in lime). The heating effect of the

gas produced may be supplemented, if need be, by resort to additional sources of heat.

Similarly as the invention is practiced upon the ashes formed in industrial furnaces, it may be performed upon the refuse of coal-mining and coal-washing operations, and upon carbonaceous shales so low in carbon content as not to justify their use as fuel. It may, indeed, be performed upon coal itself; but, ordinarily, coal of quality such as to render it serviceable as fuel will, economically, be so used; and, in consequence, the field of this invention will, in actual practice, be limited to operation upon material not generally serviceable in the industry as fuel. In case it be used upon coal, the potential heat is such in quantity that, ordinarily, it will be advantageous to add incombustible material suitable for the end in view—that is to say, lime or silica, or both.

We claim as our invention:

- 20 1. The method herein described of producing mineral wool which consists in placing carbonaceous material that contains a large proportion of mineral matter capable of being blown into wool into a slagging gas-producer, burning said material under conditions to produce producer-gas and to melt said mineral matter, conducting said gas into a steam generator and burning said gas therein to generate steam, and blowing said molten mineral matter into wool with said steam.
- 25 2. The method herein described of producing mineral wool which consists in placing carbonaceous material that contains a large proportion of mineral matter capable of being blown into wool into a slagging gas-producer, burning said material while steam is injected into it under conditions to produce producer-gas and to melt said mineral matter, conducting said gas into a steam generator and burning said gas therein to

generate steam, blowing said molten mineral matter into wool with a portion of said steam and injecting another portion of said steam into the gas-producer.

3. The method herein described of producing mineral wool which consists in placing coal ashes that contain a large proportion of mineral matter capable of being blown to wool into a slagging gas-producer, burning said coal ashes under conditions to produce producer-gas and to melt said mineral matter, conducting said gas into a steam generator and burning said gas therein to generate steam, and blowing said molten mineral matter into wool with said steam.

4. The method herein described of producing mineral wool which consists in placing in a slagging gas-producer carbonaceous material that contains a large proportion of mineral matter capable of being blown into wool, and adding flux to such material, burning said material under conditions to produce producer-gas and to melt said mineral matter and flux, conducting said gas into a steam generator and burning said gas therein to generate steam, and blowing the molten material into wool with said steam.

5. The method herein described of producing mineral wool which consists in placing in a slagging gas-producer coal ashes that contain a large proportion of mineral matter capable of being blown into wool, and adding flux to such ashes, burning the ashes under conditions to produce producer-gas and to melt said mineral matter and flux, conducting said gas into a steam generator and burning said gas therein to generate steam, and blowing the molten material into wool with said steam.

RAYMOND C. JOHNSON.  
HAROLD J. ROSE.